# EUROPEAN PATENT SPECIFICATION

(11) **EP 0 046 416 B1**
(45) Date of publication and mention of the grant of the patent: **12.11.1986**
(21) Application number: 81303806.4
(22) Date of filing: 20.08.1981
(51) Int. Cl.: B41M 1/36, B41M 5/00

(54) **Ink jet recording sheet**
Aufzeichnungsmaterial für Tintenstrahlaufzeichnung
Feuille pour l'enregistrement à jet d'encre

(30) Priority: 20.08.1980 JP 115236/80; 21.11.1980 JP 164974/80; 21.11.1980 JP 164975/80; 21.11.1980 JP 164976/80; 18.12.1980 JP 179766/80; 20.01.1981 JP 7723/81
(43) Date of publication of application: 24.02.1982
(73) Proprietor: MATSUSHITA ELECTRIC INDUSTRIAL CO., LTD., Kadoma-shi, Osaka-fu, 571 (JP)
(72) Inventor: Murakami, Mutsuaki, Kawasaki (JP); Hiromori, Yasutaka, Kuzuha Hirakata-shi Osaka (JP); Naito, Hiroshi, Machida-shi Tokyo (JP); Sekiguchi, Yumiko, Takatsu-ku Kawasaki (JP)
(74) Representative: Myerscough, Philip Boyd

## Description

This invention relates to ink jet recording sheets.

Ink jet systems are of great interest because they offer reduced noise, ease of color recording, the possibility of high speed recording, and the utilization of ordinary papers. Such systems are now being used widely in facsimile and various other types of printers. It is generally accepted that some ordinary papers can be used as recording paper in ink jet recording systems but not all ordinary papers are satisfactory. In order to obtain copies of better quality, a recording sheet should meet various requirements as follows: (1) the paper should have excellent ink receptivity to allow ink dots deposited on the paper surface to be rapidly absorbed by the paper; and (2) the paper should not allow ink dots applied to a surface to run or spread.

Requirement (1) is the most fundamental one which must be met by ink jet recording papers and assumes great importance especially when color images are produced by the ink jet system. This is because in order to produce color images, it is necessary to make a variety of colors from combinations of yellow, cyan and magenta inks, so that inks of different colors are deposited on the same portion of paper surface, resulting in large amounts of ink per unit area.

Requirement (2) is necessary for obtaining clear recorded matters. By preventing ink dots from spreading, the optical density of recorded matter can be increased. In general, the simplest method of increasing the optical density of recorded matter is to increase the concentration of dye in ink. However, this method has its limit because of the tendency of concentrated inks to clog a head nozzle. Accordingly, it is important that recording papers satisfy the above requirement.

Aside from the fundamental requirements (1) and (2), recording papers should satisfy the following further requirements: (3) the degree of penetration of an ink in the direction of depth or in the longitudinal direction should not be too great; and (4) the paper should have excellent brightness. The optical density of recorded matter largely depends on the state of the paper surface and if the degree of the penetration in the direction of depth is too great, it is difficult to make the optical density high.

The recording paper to be used in a ink jet recording system is generally made from bleached chemical pulp to which fillers, dyes and, if required, sizing agents and strength improvers are added.

There have heretofore been proposed several types of papers for ink jet recording. For instance, Japanese Laid-open Patent Application No. 52-74340 discloses an ink jet recording paper which is characterized in that a ratio of an air resistance to basis weight (g/m²) (air resistance/basis weight) is below 0.3 and that when an aqueous ink for ink jet recording is dropped in an amount of 0.004 ml, an absorption time of ink is in the range of from two seconds to 60 seconds. Further, Japanese Laid-open Patent Application No. 52-53012 teaches a method of making recording papers which is characterized by applying a coating to a base paper which has been incorporated with a wet strength improver known per se and which has a Stockigt sizing degree of below 1 second whereby the resulting surface coated paper has a Stockigt sizing degree of below 3 seconds. In these laid-open patent applications, there are described surface sizing agents including oxidized starch, PVA, galactomannon gum, polyacrylamide, sodium alginate, styrene-maleic acid copolymer, CMC and other cellulose derivatives, casein, soy bean protein and the like. In addition, there are mentioned, as sizing additives, hydrophobic materials or latices, rosin and its derivatives, petroleum resins, fumaric acid, maleic acid its derivative, waxes, synthetic resins, fatty acids, alkylketene dimers and the like, and, as pigment or filler, kaolin, calcium carbonate, aluminium hydroxide, satin white, titanium oxide, and urea-formalin organic fillers.

Moreover, there is proposed in Japanese Laid-open Patent Application No. 55-5&30 a sheet for ink jet recording which comprises a support and an ink-receptive layer formed on the surface of the support, said sheet having an opacity of 55.0 to 97.5%, an absorptivity of the ink-receptive layer being in the range of 1.5 to 18.0 mm/min. Also, Japanese Laid-open Patent Application No. 55-11829 teaches a sheet for ink jet recording which has (1) two or more layers, (2) an opacity of 55.0 to 97.5%, (3) a top layer with a thickness of 1.0 to 16.0 pm, and (4) an ink-receptivity of the top layer of 1.5 to 5.5 mm/min and that of a second layer of 5.5 to 60.0 mm/min.

The ink-receptive layer of these sheets is formed of white pigments such as clay, talc, diatomaceous earth, calcium carbonate, calcium sulfate, barium sulfate, titanium oxide, zinc oxide, zinc sulfide, satin white, aluminium silicate and lithopone. As binder resin, there are mentioned oxidized starch, etherified starch, gelatin, casein, carboxymethyl cellulose, hydroxyethyl cellulose; polyvinyl alcohol and SBR latex.

IBM Technical Disclosure Bulletin, Volume 21, No. 6, November 1978, page 2502 describes an ink jet recording sheet comprising a paper support which has been rendered water-impenetrable, to prevent ink penetration, by coating with a dielectric or water-insoluble coating, by sizing or by beating, and a water-soluble layer on the water-impenetrable paper support of a polymer such as polyvinyl alcohol, starch, gelatine or polyvinyl pyrrolidone.

We have made extensive studies of ink jet recording papers which satisfy the afore-mentioned requirements (1) to (4) and found that papers made using combinations of sizing agent or binding agent resins and pigments and fillers which have been known from the Laid-Open Patent Applications do not show satisfactory characteristics when applied for such recording purpose. Especially, the resins serving as the sizing agent or binding agent play an important role and it has been found that the known resins are unsatisfactory in ink receptivity and thus recorded matter using such resins as a surface coating frequently shows insufficient optical density.

The present invention seeks to provide a jet recording sheet which shows an improved optical density, when recorded, over known sheets, which shows an excellent ink receptivity and is able to suppress ink dots from spreading, and which can ensure a certain extent of water-proofing and excellent fastness of light of recorded matter.

According to the present invention, there is provided a recording sheet for ink jet recording which comprises a water-penetrable paper support to at least one surface of which has been applied an aqueous dispersion comprising, as binding agent, polyvinylpyrrolidone, vinylpyrrolidone-vinyl acetate copolymer or a mixture thereof and a white filler, the weight ratio of said white filler to said binding agent being from 10:1 to 0.2:1, or which comprises a water-penetrable paper sheet prepared from a mixture of 100 parts by weight of a paper-making pulp and an aqueous dispersion comprising, as sizing agent, 2 to 20 parts by weight of polyvinylpyrrolidone, vinylpyrrolidone-vinyl acetate copolymer or a mixture thereof and 10 to 60 parts by weight of a white filler, the aqueous dispersion in each case comprising, as water-proofing agent, an aqueous emulsion-type resin or an alcohol-soluble resin which forms a water-proof film upon drying, in an amount of 1 to 50 wt% of the total weight of the resins used as water-proofing and binding or sizing agents.

As having described hereinabove, one of features of the present invention resides in use of polyvinylpyrrolidone (hereinafter abbreviated as PVP) and/or vinylpyrrolidone-vinyl acetate copolymer (hereinafter abbreviated as PVPNAc). The PVP and PVPNAc are water-soluble polymers and have a film-forming property. They are industrially applied as cosmetics, medical supplies, adhesives, cleaning agents and soaps, fiber-finishing agents, and inks, and also in the field of lithographic printing and paper. PVP and PVP/ VAc which are applied in the field of the paper-making industry are used as a decoloring agent for rags for regeneration, an improver of cellulose paper to improve its tensile strength, and a binder for the specific type of paper made of inorganic flakes or fibers.

When applied to inks making use of dyes, PVP renders the dye more readily soluble, serves to prevent gelation, and imparts deep color tone even to inks of low dye concentration.

PVP and PVPNAc are soluble in water and have generally an average molecular weight of several thousands to several hundred thousands. These polymers may be prepared by any known technique.

The commercially available vinylpyrrolidone and vinyl acetate copolymer has a ratio of PVNAc generally in the range of 70/30 to 30/70.

The PVP and/or PVA/VAc is used in the practice of the invention together with a white pigment or filler. Examples of the filler which is preferably used in combination with the PVP resin or PVPNAc copolymer as will become apparent from examples appearing hereinafter include clay, talc, calcium carbonate, calcium sulfate, calcium silicate diatomaceous earth, magnesium silicate, terra alba, activated clay, magnesium oxide, magnesium carbonate and aluminium hydroxide. Aside from these, fillers which are ordinarily employed in the paper-making industry such as titanium oxide, silica, aluminium silicate, satin white and zinc oxide may be used though they are inferior in optical density and other characteristics to those mentioned above.

In one aspect of the invention, an aqueous dispersion of the binding agent, the water-proofing agent and the filler is applied onto at least one surface of the paper support. The weight ratio of the filler to the binding agent is generally 10:1 to 0.2:1, preferably 1:1 to 1:2. This will be particularly described in examples appearing hereinafter. The aqueous dispersion is applied to a paper support, which may be any paper ordinarily employed for ink jet recording purpose, in an amount of 3 to 50,g/m² on the dry basis. Preferably, the coating amount is from 10 to 30 g/m² and most preferably about 20 g/_{M}².

In order to improve water proofing, the PVP and/or PVPNAc binding agent resin may be mixed with a water-soluble sizing agent or binder which is ordinarily employed in the paper-making industry, including, for example, oxidized starch, PVA, styrene-maleic acid copolymer, carboxymethyl cellulose (CMC), and hydroxyethylcellulose. When the mixture is used, the PVP and/or PVPNAc binding agent resin should be contained in an amount of not smaller than 20 wt% of the mixture.

When it is desired to control the hardness of the PVPNAc film, there may be added to the aqueous dispersion as usual plasticizers such as dimethyl phthalate, glycerine, diethylene glycol, sorbitol allyl- sulfonamide-formaldehyde, cellulose butyrate and cellulose butyrate-propionate.

In another aspect of the present invention, the aqueous dispersion is mixed with stock pulp and then an ink i-at recording paper is made from the mixture by any known paper-making technique. The paper incorporating therein the PVPNAc resin, the water-proofing agent and filler composition has several advantages: The making process is simple; and the PVP or PVPNAc is readily soluble in water and is thus poor in water proofing, so that when a PVP or PVPNAc-coated paper is dipped in water, the coating layer is readily dissolved out but the internally incorporated paper has a certain degree of water proofing though the filler comes off from the paper when dipped in water. This is experimentally confirmed that when a surface coated recording paper is vertically dipped in water, a coating layer composed of PVP or PVPNA_{C} and white filler comes off from the paper support in 5 to 10 seconds. On the other hand, even when the internally incorporated recording paper is dipped in water for 10 seconds, only several percent of filler is found to come off from the paper. In addition, it takes over one minute before the pulp stock of the paper itself is reduced into pieces and dispersed in water. As a matter of course, such a time varies depending on the amount of PVP or PVPNAc. A reason why the water proofing is improved by internally applying the composition is believed due to the fact that the resin or binder component is uniformly mixed with a pulp component and thus the speed of infiltration of water becomes slow and no coating layer is come off as will be experienced in the case of the surface coating.

The internally applied recording paper can be made by one step without involving an additional coating process and is thus much simpler in manufacturing step than the surface-coated recording paper.

However, the resin and filler are usually present in amounts greater than those required for the surface coating technique. That is, as defined hereinbefore, the PVP and/or PVPNAc is used in an amount of 2 to 20 parts by weight and a white filler is used in an amount of 10 to 60 parts by weight both per 100 parts by weight of stock pulp. The amount of the white filler, of course, varies more or less depending on the type of the filler.

The water-proofing of either type of recording paper is much improved by the presence in the aqueous dispersion of, as water-proofing agent, the aqueous emulsion-type resin or a polymer soluble in alcohol which is capable of forming a water-proof film after drying. Water-soluble resin binders such as oxidized starch, PVA, CMC and hydroxyethyl cellulose serve to improve the water-proofing as described hereinbefore when used in combination with PVP or PVPNAc but are not essential for such purpose. For instance, the coating layer obtained from the mixture of a water-soluble resin binder and PVP or PVPNAc is dissolved in water in 10 to 15 seconds and an increasing amount of the water-soluble resin binder gives an adverse influence of ink receptivity.

Examples of the aqueous emulsion useful in the practice of the invention are those of polyvinyl acetate, ethylene-vinyl acetate copolymer (having an ethylene content of below 30%), acrylic esters and water-soluble shellac. Examples of polymers soluble in alcohol include polyvinyl butyral, polyacrylamide, polyamide-epichlorohydrin, shellac and polyvinyl acetate. These resins are capable of forming films of relatively good water proofing after drying. The amount of these resins is in the range of 1 to 50 wt%, preferably 2 to 20 wt%, of a mixture of the resin and PVP or PVPNAc.

In addition to these resins, various additives may be added to the PVP or PVPNAc and filler. In particular, the resistance or the fastness to light of recorded matter is one of important problems to solve.

Then, we have made an intensive study on the light fastness or resistance. The most general way of improving the fastness to light of recorded matter is to use dyes which have excellent fastness to light. However, since inks to be employed in the ink jet recording system should not cause clogging of ink jet nozzles and should have a clear color tone, dyes with excellent light fastness cannot always be employed. Basic dyes, acid dyes, or mordant dyes are clear in color tone and are now widely used for the ink jet recording purpose but these dyes are not necessarily excellent in light fastness.

The light fastness of recorded matter can be improved by adding to the aqueous dispersion of PVP and/ or PVPNAc, water-proofing agent and filler (1) antioxidants, (2) UV absorbers and (3) metal oxides, metal chlorides or tannic acid capable of reacting with dyes to convert the dyes into light-fast dyes.

During the course of our study, we have found that though the light fastness more or less depends on the type of dye, the light fastness of recorded matter is poorer than that of dye in liquid state and fading is mainly caused by photooxidation brought about by oxygen in air and light. To prevent this, antioxidants have been found to be effective. Moreover, an investigation was conducted to known the mechanism of the fading in relation to wavelength. That is, glass filters were used to select desired ranges of wavelength and a Xenone fade meter was used to measure the resistance to light of recorded matter. As a result, it was found (1) that little fading took place in the wavelength range of infrared rays, (2) that in the range of visible light, fading occurred in a wavelength corresponding to a main absorption peak of dye; (3) that fading by the ultraviolet light was as great as in (2).

For instance, a magenta ink composed of 79% of water, 20% of ethylene glycol and 11 % of Basic Violet showed light resistance as follows.

From the results, it was considered that UV absorbers were effective to prevent fading of recorded matter, which was experimentally found true.

These antioxidants, UV absorbers, and compounds capable of converting dyes into light-resistant dyes or pigments are suitably used in amounts of 0.1 to 10 wt% of a mixture of the PVP or PVPNAc and filler. Among dyes that can be employed in inks for use with the recording papers of the invention are C.I. Basic Yellow 11, C.I. Basic Red 1, C.I. Basic Red 3, C.I. Basic Violet 14, C.I. Basic Blue 3, C.I. Mordant Orange 4, C.I. Mordant Red 15, C.I. Mordant Violet 5, C.I. Mordant Black 7, C.I. Acid Yellow 17, C.I. Acid Orange 7, C.I. Acid Red 88, C.I. Acid Violet 49, C.I. Acid Blue 7, C.I. Acid-Black 2, C.I. Acid Black 31, C.I. Basic Yellow 11, C.I. Basic Red 13, C.I. Basic Yellow 17, C.I. Direct Yellow 50 and C.I. Direct Red 80. Inks containing these dyes can be composed of 76 or 77 to 79 percent by weight of water, 20 percent of ethylene glycol and 1 to 3 or 4 percent by weight of the dye.

The present invention will now be further described by way of Examples. In experiments carried out in connection with the invention four types of PVP were used having average molecular weights of 360,000 (hereinafter referred to as K-90), 160,000 (hereinafter referred as K-60), 40,000 (hereinafter referred to as K-30) and 10,000 (hereinafter referred to as K-10) but little or no substantial difference in recording characteristics was observed among them and K-30 was used as the representative PVP in the examples. In addition, four types of PVPNAc having VPNAc ratios of 70/39, 60/40, 50/50 and 30/70, respectively, were used to check recording characteristics. As a result it was found that good results were obtained in each case without showing any significant differences among them. Accordingly, a PVPNAc resin having a VP/ VAc ratio of 50/50 was used in the Examples as the representative PVPNAc.

The ink jet recording was carried out using an On-demand-type head with a diameter of nozzle of 40 µm in which three ink jetting heads were used to discharge therefrom different types of inks including cyan, yellow and magenta. By the combination of these inks, different colors of red, green, blue and sepia were made. The discharge of ink was changed in seven stages by controlling an application voltage and the recording of 6 lines/mm was conducted. In the case of monochrome, amounts of discharge per unit area in the respective stages are 2.6 x 10-⁴ cc/cm² in first stage, 4.7 x 10-⁴ cc/cm² in second stage, 6.4 x 10-⁴ cc/ cm² in third stage, 7.0 x 10-⁴ cc/cm² in fourth stage, 7.9 x 10-⁴ cc/cm² in fifth stage, 8.7 x 10-⁴ cc/cm² in sixth stage, and 9.4 x 10-⁴ cc/cm² in seventh stage, respectively. In the case of blue in color, the amounts of discharge in the respective stages become double and in the case of sepia color, they become three times. Accordingly, the severest recording conditions are those for the sepia color in the seventh stage. Aside from these recordings, a recording of 2 lines/mm was also conducted for comparison.

Recorded matters were evaluated according to the following measurements or observations: (1) Measurement of optical density of the respective colors in the seventh stage; (2) Judgement of a stage of sepia color where inks start to run or spread so as to check a degree of the running or spreading of the inks (which show a degree of ink receptivity of paper); (3) Measurement of a time before the sepia color of the seventh stage is apparently dried after application thereof; and (4) Measurement of a rate of area of recorded matter of the first stage in which two lines/mm were recorded (to know a degree of spreading of ink dots or a degree of so-called sharpness).

### Example 1

In this example, calcium carbonate was used as a white pigment and different types of binder resins were used including PVP and PVPNAc to be used in the present invention.

To a 5% aqueous solution or dispersion of each binder resin was added 15 wt% of calcium carbonate of a powder form having a size of 0.1 to 0.2 pm, followed by fan agitating to give a slurry. This slurry was applied onto a commercially available groundwood paper by means of a wire bar, followed by roll pressing to obtain a surface-coated paper. The coated paper had a thickness of 5 to 20 µm, i.e. 0.3-2.0 g of the coating was applied onto an A-4 size paper.

The respective recording papers thus made were subjected'to the recording procedure and evaluated according to the measuring methods described hereinabove. The test results are shown in Table 1.

In this table, the optical density was determined with respect to the magenta color of the seventh stage and other six colors showed a similar tendency.

As will be clearly seen from the results of Table 1, the binder resin gives a great influence on the characteristics of ink spreading, drying time and the like and the PVPNAc resins involve no spreading or running at the seventh stage and are thus much better than the other binder resins. PVA and hydroxyethyl cellulose rank second to PVP and PVPNAc with respect to optical density but these resins were inferior in spreading characteristic, i.e. spreading occurred at the sixth stage, and required a drying time of as long as 60 to 80 seconds. As to the optical density and rate of area, oxidized starch was excellent and PVP and PVP/ VAc showed such characteristics next to oxidized starch.

### Example 2

In this example, PVP and PVP/VAc were used as a binder resin and different types of white pigments were used in combination for comparative purpose.

To a 10% aqueous solution of PVP or PVPNAc was added each of white pigments to be tested to give a slurry in the same manner as in Example 1 and the slurry was applied in the same manner as in Example 1 to obtain a surface coated paper. The type and amount of white pigment and the results of recorded matter are shown in Table 2 below with regard to the PVP binder resin.

As will be appreciated from the results of Table 2, with titanium oxide, silica, aluminium silicate, satin white and zinc oxide, there appears a whitely fading phenomenon where an entirety of image is observed as white and the optical density does not become higher than 0.9. This is because an ink does not remain on the surface of the coated paper and the white pigment deposits out on the paper surface. In contrast thereto, clay, talc, calcium carbonate, calcium sulfate, calcium silicate, diatomaceous earth and aluminium hydroxide show no fading phenomenon and optical densities of above 0.9. The white pigments causing the fading phenomenon cannot be used in large amounts and do not show an effect of increasing the whiteness of paper though usable in the practice of the invention. In this sense, the white pigments showing no fading phenomenon are conveniently and preferably used. Preferable pigments further include magnesium silicate, terra alba, activated clay, magnesium oxide and magnesium carbonate. As regards the spreading characteristic and drying time, there is not a significant difference depending on the type of pigment, revealing that such characteristics are mainly dependent of the type of binder.

In Table 2, the binder used was PVP and similar results were obtained when PVPΛIAc was used except that the optical density was reduced by about 0.5 in all the cases.

### Example 3

In this example, PVP was used as binder resin and calcium carbonate, calcium silicate and talc were used as pigment to determine an effect of a ratio by weight of the binder and the white pigment on the recording characteristics. The coated paper was made in the same manner as in Example 1. In Table 3, there are shown results of a test using calcium carbonate.

As will be clear from the results of Table 3, high optical density cannot be obtained when amounts of PVP and calcium carbonate are too great or too small. That is, in order to obtain good recording characteristics, a PVP/calcium carbonate (with an average size of 0.1 to 0.2 pm) ratio by weight is preferably in the range of 10:1 1 to 0.25:1. When a similar test was conducted using a calcium silicate powder having an average particle size of 0.1 pm and a talc powder having an average size of 0.2 to 0.3 µm, it was found that a preferable weight ratio was in the range of 10:1 to 0.5:1 for calcium silicate and 5:1 to 0.2:1 for talc. The weight ratio is, of course, dependent on the size of white pigment and the weight ratio of PVP or PVPNAc and a white pigment is conveniently in the range of 10:1 to 0.2:1.

Furthermore, when the composition comprising calcium carbonate and PVP was applied in different thicknesses ranging from 4 pm to 28 µm, no significant difference in recording characteristics was found in this range of thicknesses.

In addition, four types of paper support showing different water absorptivities were used to check their influence on the recording characteristics. As a result, it was found that when the coated layer had a thickness of above 8 µm, inclusive, good results were obtained in any cases.

From the above, the coated layer should preferably have a thickness of 8 µm or more, and the coating composition of the invention can be widely applied to a wide variety of paper supports.

### Example 4

In this example, PVP and other binder resins were used in combination. As a white pigment, talc (Chinese talc) were used. Amounts of the binder resin and talc were, respectively, 20%. Coated papers were made substantially in the same manner as in Example 1, with the results summarized in Table 4 below.

As will be appreciated from the above results, binder resins such as PVA, oxidized starch and the like show better ink receptivity when used in combination with PVP.

A greater amount of PVP is desirable in view of the ink receptivity. Though the content of PVP depends on the type of the second binder, it is in the range of over 20 wt% when the binder resin used in combination with PVP shows water absorptivity such as PVA and in the range of 33 wt% when the second binder resin shows no water absorptivity.

### Example 5

In this example, characteristics of ink. jet recording papers made by a size press technique are described.

Different types of binder and calcium carbonate were mixed in a ratio of 1:1 in an aqueous medium to obtain 10% slurries. Each slurry was coated on a commercially available groundwood paper by a size press system to obtain a surface coated paper with a coating spread of 4.0 g/m². The results are shown in Table 5 below.

From the above results, it will be seen that the characteristics of the recording papers made by the size press technique are substantially the same as those of the recording papers obtained by the wire bar. For instance, the recording paper of the coated type using PVP/VAc as binder had an optical density of 0.99, a spreading stage of >7, a drying time of <10, and a rate of area of <10 as shown in Table 1, which are almost the same as those of Table 5. In the PVP/PVA and PVP/oxidized starch systems, the recording characteristics are almost the same as those of Table 4. Accordingly, the size press technique can be used similarly with the surface coating method.

### Example 6

In this example, resins used as sizing agents or binders and calcium carbonate used as white pigment were applied internally or mixed with pulp.

LBKP and NBKP were mixed in a ratio of 1:2 and beaten in a refiner. Then, light calcium carbonate was added to the pulp in an amount of 30 parts by weight per 100 parts by weight of the pulp and PVP or PVP/ VAc was added in an amount of ranging from 0.5 to 30 wt% based on the pulp. The pulp composition was subjected to a paper-making process using a Fourdriner test machine to make a paper with a basis weight of 70 g/m². The thus made papers were each subjected to the calender rolls to give recording papers.

The recording papers were applied with inks and evaluated in the same manner as described hereinbefore, with the result shown in Table 6 below.

In the table, the optical density is obtained from the magenta color of the seventh stage and as regards the other six colors, a similar tendency is observed.

As will be appreciated from the above results, where the binder content is 0.5% or 1 %, the optical density, stage where spreading appeared, drying time and rate of area are not satisfactory. Accordingly, the binder resin should be contained in an amount of at least 2% of the pulp. This is much larger as compared with an amount of an strength improver ordinarily employed in the paper-making industry (generally in the range of 0.2 to 1 wt%). On the other hand, the recording papers in which 30% of PVP or PVPNAc based on the pulp is contained show excellent recording characteristics but become sticky to the touch. In addition, such papers show a blocking tendency.

Gathering the above, the content of PVP or PVPNAc is in the range of 2 wt% to 20 wt% of the pulp.

### Example 7

In this example, an amount of PVP was set at 10% by weight of pulp but an amount of calcium was changed. Recording papers were each made and evaluated in the same manner as in Example 6. The test results are shown in Table 7 below.

As will be apparent from the above results, good recording characteristics are obtained when the content of the white filler is in the range of 10 to 60 wt% of the pulp. Less contents are disadvantageous in that the optical density is poor while larger contents lead to the whitely fading phenomenon. Accordingly, an effective amount of calcium carbonate is in the range of 10 to 60 wt% of the pulp. In this connection, the content of calcium carbonate more or less depends on the content of PVP, e.g. when the content of PVP is 2%, the upper limit in content of calcium carbonate was found to be 40%. Similar results were obtained when PVPNAc was used instead of PVP.

The above procedure was repeated using other several white pigments in different amounts. As a result, it was found that a suitable content of clay was in the range of 10 to 60 wt% of the pulp, that of talc ranged from 10 to 60 wt%, that of calcium sulfate ranged from 5 to 40 wt%, that of calcium silicate ranged from 10 to 40 wt%, that of diatomaceous earth ranged from 10 to 60 wt%, that of satin white ranged from 5 to 50 wt%, and that of zinc oxide ranged from 15 to 40 wt%. Generally speaking, white pigments are effectively usable in the range of 10 to 60 wt% of pulp. Other usable white pigments in this internal application technique are aluminium hydroxide, silica, aluminium silicate, magnesium silicate, terra alba, activated clay, magnesium oxide, magnesium carbonate and aluminium oxide. Among the white pigments, preferable ones are those mentioned with respect to the surface coating method.

The following three examples illustrate water-proof, film-forming resins added to the basic composition used in the present invention.

### Example 8

In this example, binder resin made of 90 parts by weight of PVP and 10 parts by weight of different types of film-forming polymers were used.

To 10% aqueous or alcoholic solutions of various binder resin mixtures was added calcium carbonate powder with a size of 0.1 to 0.2 ₁₁m in an amount of as great as three times the binder resin mixture, followed by agitating with a fan to give slurries. Each slurry was applied onto a commercially available groundwood paper by a wire bar and the thus applied paper was roll pressed to obtain surface coated papers. The thickness of the coated layer was in the range of 5 to 20 pm. The thus obtained papers were recorded and evaluated in the same manner as in Example 1 except for water proof. That is, the water proof was equated as follows: a time before the coated layer was completely separated from a coated paper specimen with a size of 1 cm x 2 cm after having immersed the coated paper vertically in water was measured. The test results are shown in Table 8 below.

From the above results, it will be appreciated that when PVP or PVPNAc is used singly, the water proof is 5 seconds or less. In addition, systems of PVP or PVPNAc to which other water-soluble polymers such as oxidized starch, PVA and hydroxyethyl cellulose have been added show a slight improvement in water proof. On the other hand, binder resin mixtures in which 10 wt% of aqueous emulsion-type polymers such as polyvinyl acetate, ethylene-vinyl acetate copolymer, acrylic ester resin and water-soluble shellac show a water proof of over 25 seconds, thus improving the water proof remarkably. These binder resin mixtures are slightly inferior in recording characteristics, i.e. the spreading stage of seven and a drying time of 13-19, to the PVP or PVPNAc resin alone. However, these slight degrees of deterioration of the characteristics are almost negligible and the improvement in water proof is much more effective. Similar results are obtained when polyvinyl butyral, polyacrylamide, polyamide - epichlorohydrin and shellac are used as dissolved in methanol solvent.

Aside from the resins mentioned above, other resins are also usable in combination with PVP and/or PVPNAc including vinyl acetate-acrylonitrile copolymer, styrene resin, styrene-acrylonitrile copolymer, methacrylic ester resin, polyamide resin, melamine resin and melamine-urea resin.

### Example 9

In this example, an influence of polyvinyl acetate in a binder resin composed of PVP and polyvinyl acetate was checked. To an aqueous 10% solution of the binder resin was added talc (Chinese talc) i an amount of two times the binder resin to give a slurry. Then, Example 8 was repeated with the results shown in Table 9.

As will clear from the above results, the proof to water improves as the amount of polyvinyl acetate is increased. However, the optical density, spreading characteristic and drying time become worse with an increasing amount of polyvinyl acetate. For instance, the drying time is 49 seconds for the binder system of PVP/polyvinyl acetate = 40/60. This time is longer than the time between completion of image formation and withdrawal of the recorded matter from a machine and is not thus practical. Taking the above into consideration, a maximum amount of polyvinyl acetate should be 50%, i.e. it is necessary that polyvinyl acetate does not exceed that of PVP. On the other hand, the binder system containing 2% of polyvinyl acetate does show little effect and thus polyvinyl acetate should be over 2%.

The above procedure was repeated using different types of film-forming and water-proof polymers to determine the range of addition of each polymer which may more or less depend on the type and amount of white pigment, and thickness of the coated layer. The results are shown in Table 10.

From the above results, is is generally possible to use these water proof-imparting resins in the range of 1 to 50 wt% of the mixture with PVP or PVPNA_{C} provided that the type and amount of white pigment and the thickness of the coated layer are properly controlled.

### Example 10

In this example, characteristics of ink jet recording papers made by the size press technique are shown.

Various binders (PVP: additive polymer = 90:10) and calcium carbonate were mixed in a weight ratio of 1:2 to give 10% slurries. Each slurry was applied onto a commercially available groundwood paper by the size press method in an amount of 4.0 g/m² on a dry basis to give a surface coated paper. The thus obtained coated papers had recording characteristics shown in Table 11.

As will be clearly seen from the above results, the characteristics of the recording papers made by the size press method are excellent similarly to those of the recording papers made by the wire bar coating method. As for the water proof, the recording papers made by the size press method are slightly superior to those obtained by the wire bar coating method. Thus, the size press technique can be used similarly with the surface coating method.

The following examples deal with the manner of imparting light resistance to recorded matter in which antioxidants, Ultraviolet absorbers and compounds capable of reacting with dyes for conversion into light-resistant dyes.

The measurement of light resistance was conducted according to the method as prescribed in JIS L0843-71 using a 2.5 KW xenon fade meter of an air-cooling type (made by Suga Tester K.K.). The irradiation energy was 464 J/cm². Hr, which is 9.6 times that of an average sunlight and 380 times that of a fluorescent lamp.

The ink jet recording was carried out using an On-demand-type head having a nozzle diameter of 40 µm and a voltage of 200 V was applied to the recording system. When a recording of 6 lines/mm² was effected, a discharge per unit area was 7.9 x 10-⁴ cc/cm².

Recording papers used were made by applying onto a commercially available high quality paper a coating composition comprising polyvinyl alcohol/polyvinylpyrrolidone (40/60) as binder and calcium carbonate as white filler in a binder-to-filler weight ratio of 1:1. The coating amount was 40 g/m². Antioxidants, UV absorbers and the specific type of compounds capable of reacting with dyes were dissolved in the binder to make recording papers.

### Example 11

Various metal oxides and organic acids were added to the binders in such an amount that they were contained in the surface coating in an amount of 0.5 g/m². Then, recording papers were made substantially in the same manner as in the foregoing Examples.

Then, a magenta ink made of 79% by weight of water, 20% by weight of ethylene glycol and 1 % by weight of C.I. Basic Violet 10 was prepared and used for recording on the respective recording papers. The recorded papers were irradiated for 12 hours in the xenone fade meter and their optical density was measured. The test results are shown in Table 12 below.

As will be seen from the above results, the additives remarkably improve the light resistance of recorded matter. In practice, the phosphorus-containing acids are preferred because of their excellency in color retentivity.

### Example 12

Example 11 was repeated using various antioxidants, with the results shown in Table 13 below.

These results reveal that the addition of antioxidants can remarkably improve the light resistance. The degree of improvement depends on the type of antioxidant, but hydroquinone, p-tert-butylcatechol, 2,6-di- tert-butylphenol and methylhydroquinone have been found to be particularly good in improving light resistance.

Aside from those antioxidants mentioned above, there are usable styrenated phenol, 2,2'-methylene- bis(4-ethyl-6-t-butylphenol), 4,4'-butylidenebis(3-methyl-6-t-butylphenol), 4,4'-thiobis(3-methyl-6-t-butylphenol), 2,2'-thiobis(4-methyl-6-t-butylphenol), alkylthiodipropionates, 2-mercaptobenzoimidazole, N-n-butyl-p-aminophenol, phenylenediamines, a-naphthylamine, N-phenyl-a-naphthylamine, N,N'- disalicylidene-1,2-propylenediamine, phenothiazine, tris(nonylphenyl)phosphite, triphenylphosphite, tris(3,5-di-t-butyl-4,4-hydroxyphenylphosphate, dithiocarbamate, anthogenate, dihydroquinoline derivatives, mercaptobenzimidazoles, monoisopropyl citrate, ethyl protocathecuate, alkyl gallates, nor- dihydroguaiaretic acid and L-sorbic acid.

### Example 13

Example 11 was repeated using various UV absorbers, with the results shown in Table 14 below.

These results show that the addition of the UV absorbers is effective in improving the light resistance.

## Claims

1. An ink jet recording sheet which comprises a water-penetrable paper support to at least one surface of which has been applied an aqueous dispersion comprising, as binding agent, polyvinylpyrrolidone, vinylpyrrolidone-vinyl acetate copolymer or a mixture thereof and a white filler, the weight ratio of said white filler to said binding agent being from 10:1 to 0.2:1, or which comprises a water-penetrable paper sheet prepared from a mixture of 100 parts by weight of a paper-making pulp and an aqueous dispersion comprising, as sizing agent, 2 to 20 parts by weight of polyvinylpyrrolidone, vinylpyrrolidone-vinyl acetate copolymer or a mixture thereof and 10 to 60 parts by weight of a white filler, the aqueous dispersion in each case comprising, as water-proofing agent, an aqueous emulsion-type resin or an alcohol-soluble resin which forms a water-proof film upon drying, in an amount of 1 to 50 wt% of the total weight of the resins used as water-proofing and binding or sizing agents.

2. An ink jet recording sheet according to claim 1, wherein said dispersion has been applied to a surface of the paper support in an amount of 3 to 50 g/m² on a dry basis.

3. An ink jet recording sheet according to claim 1 or 2, wherein said filler is a powder of clay, talc, calcium carbonate, calcium sulfate, calcium silicate, diatomaceous earth, magnesium silicate, terra alba, . activated clay, magnesium oxide, magnesium carbonate or aluminium hydroxide.

4. An ink jet recording sheet according to claim 1, 2 or 3, wherein the aqueous dispersion also comprises a water-soluble resin, the binding or sizing agent resin being used in an amount of at least 20 wt% of the total weight of said resins.

5. An ink jet recording sheet according to any one of the preceding claims, wherein the aqueous dispersion comprises a plasticizer to control the hardness of a film formed from the resin used as binding or sizing agent.

6. An ink jet recording sheet according to any one of the preceding claims, wherein the aqueous dispersion comprises 0.1 to 10 wt% of an antioxidant, UV absorber or compound capable of reacting with a dye.

7. An ink jet recording sheet according to claim 6, wherein the antioxidant, UV absorber or compound capable of reacting with a dye is contained at least in a surface layer of the recording sheet.

8. An ink jet recording sheet according to claim 6, wherein the antioxidant, UV absorber or compound capable of reacting with a dye is contained in the recording sheet.

9. An ink jet recording sheet according to claim 6, 7 or 8, wherein the compound capable of reacting with a dye is a phosphorus tungstic acid, a phosphorus molybdic acid or a phosphorus tungsten molybdic acid.

10. An ink jet recording sheet according to any one vf the preceding claims wherein the weight ratio of said white filler to said binding agent is from 1:1 to 2:1.

## Patentansprüche

1. Blattförmiges Aufzeichnungsmaterial für Tintenstrahlaufzeichnung, das aus einem wasserdurchlässigen Träger aus Papier besteht, wobei auf mindestens eine Oberfläche des Trägers eine wäßrige Dispersion aufgebracht worden ist, die Polyvinylpyrrolidon, Vinylpyrrolidon-Vinylacetat-Copolymer oder eine Mischung davon als Bindemittel und einen weißen Füllstoff enthält, und wobei das Masseverhältnis des erwähnten weißen Füllstoffs zu dem erwähnten Bindemittel 10:1 bis 0,2:1 beträgt, oder das aus einem wasserdurchlässigen Papierblatt besteht, das aus einer Mischung von 100 Masseteilen eines Papierrohstoffs und einer wäßrigen Dispersion, die 2 bis 20 Masseteile Polyvinylpyrrolidon, Vinylpyrrolidon-Vinylacetat-Copolymer oder einer Mischung davon als Leimungsmittel und 10 bis 60 Masseteile eines weißen Füllstoffs enthält, hergestellt wird, wobei die wäßrige Dispersion in jedem Fall als wasserdichtmachendes Mittel ein Harz vom Typ einer wäßrigen Emulsion oder ein alkohollösliches Harz, das beim Trocknen einen wasserdichten Film bildet, in einer auf die Gesamtmasse der als wasserdichtmachendes Mittel und der als Bindemittel oder Leimungsmittel verwendeten Harze bezogenen Menge von 1 bis 50 Masse% enthält.

2. Blattförmiges Aufzeichnungsmaterial für Tintenstrahlaufzeichnung nach Anspruch 1, bei dem die erwähnte Dispersion in einer Menge von 3 bis 50 g/m² (Bezugsbasis Trockenmasse) auf eine Oberfläche des Trägers aus Papier aufgebracht worden ist.

3. Blattförmiges Aufzeichnungsmaterial für Tintenstrahlaufzeichnung nach Anspruch 1 oder 2, bei dem der erwähnte Füllstoff ein Pulver von Ton, Talk, Calciumcarbonat, Calciumsulfat, Calciumsilicat, Kieselgur, Magnesiumsilicat, Kaolin, aktiviertem Ton, Magnesiumoxid, Magnesiumcarbonat oder Aluminiumhydroxid ist.

4. Blattförmiges Aufzeichnungsmaterial für Tintenstrahlaufzeichnung nach Anspruch 1, 2 oder 3, bei dem die wäßrige Dispersion auch ein wasserlösliches Harz enthält, wobei das als Bindemittel oder Leimungsmittel verwendete Harz in einer auf die Gesamtmenge der erwähnten Harze bezogenen Menge von mindestens 20 Masse% verwendet wird.

5. Blattförmiges Aufzeichnungsmaterial für Tintenstrahlaufzeichnung nach einem der vorhergehenden Ansprüche, bei dem die wäßrige Dispersion ein Plastifizierungsmittel enthält, um die Härte eines Films zu steuern, der aus dem als Bindemittel oder Leimungsmittel verwendeten Harz gebildet wird.

6. Blattförmiges Aufzeichnungsmaterial für Tintenstrahlaufzeichnung nach einem der vorhergehenden Ansprüche, bei dem die wäßrige Dispersion 0,1 bis 10 Masse% eines Antioxidationsmittels, eines UV-Absorptionsmittels oder einer zum Reagieren mit einem Farbstoff befähigten Verbindung enthält.

7. Blattförmiges Aufzeichnungsmaterial für Tintenstrahlaufzeichnung nach Anspruch 6, bei dem das Antioxidationsmittel, das UV-Absorptionsmittel oder die zum Reagieren mit einem Farbstoff befähigte Verbindung mindestens in einer Oberflächenschicht des blattförmigen Aufzeichnungsmaterials enthalten ist.

8. Blattförmiges Aufzeichnungsmaterial für Tintenstrahlaufzeichnung nach Anspruch 6, bei dem das Antioxidationsmittel, das UV-Absorptionsmittel oder die zum Reagieren mit einem Farbstoff befähigte Verbindung in dem blattförmigen Aufzeichnungsmaterial enthalten ist.

9. Blattförmiges Aufzeichnungsmaterial für Tintenstrahlaufzeichnung nach Anspruch 6, 7 oder 8, bei dem die zum Reagieren mit einem Farbstoff befähigte Verbindung eine Wolframatophosphorsäure, eine Molybdatophosphorsäure oder eine Wolframatomolybdatophosphorsäure ist.

10. Blattförmiges Aufzeichnungsmaterial für Tintenstrahlaufzeichnung nach einem der vorhergehenden Ansprüche, bei dem das Masseverhältnis des erwähnten weißen Füllstoffs zu dem erwähnten Bindemittel 1:1 bis 2:1 beträgt.

## Revendications

1. Feuille pour enregistrement à jet d'encre qui comprend un support de papier pénétrable par l'eau, dont au moins une surface a été enduite d'une dispersion aqueuse comprenant, comme agent liant, de la polyvinylpyrrolidone, un copolymère (vinylpyrrolidone/acétate de vinyle) ou un de leurs mélanges et une charge blanche, le rapport pondéral de la dite charge blanche au dit agent liant étant de 10:1 à 0,2:1, ou qui comprend une feuille de papier pénétrable par l'eau préparée à partir d'un mélange de 100 parties en poids de pâte à papier et d'une dispersion aqueuse comprenant, comme agent d'encollage, 2 à 20 parties en poids de polyvinylpyrrolidone, d'un copolymère (vinylpyrrolidone/acétate de vinyle) ou d'un de leurs mélanges, et 10 à 60 parties en poids d'une charge blanche, la dispersion aqueuse comprenant dans chaque cas, comme agent imperméabilisant à l'eau, une résine du type émulsion aqueuse ou une résine soluble dans les alcools qui forme, au séchage, un film imperméable à l'eau, à raison de 1 à 50% en poids du poids total des résines utilisées comme agents d'imperméabilisation à l'eau et comme liants ou agents d'encollage.

2. Feuille pour enregistrement à jet d'encre selon la revendication 1, dans laquelle la dite dispersion a été appliquée sur une surface du support de papier à raison de 3 à 50 g/m² sur une base sèche.

3. Feuille pour enregistrement à jet d'encre selon la revendication 1 ou 2, dans laquelle la dite charge est une poudre d'argile, de talc, de carbonate de calcium, de sulfate de calcium, de silicate de calcium, de diatomite, de silicate de magnésium, de kaolin, d'argile activée, d'oxyde de magnésium, de carbonate de magnésium ou d'hydroxyde d'aluminium.

4. Feuille pour enregistrement à jet d'encre selon la revendication 1, ou 3, dans laquelle la dispersion aqueuse comprend aussi une résine hydrosoluble, la résine servant de liant ou d'agent d'encollage étant utilisée à raison d'au moins 20% en poids du poids total des dites résines.

5. Feuille pour enregistrement à jet d'encre selon l'une quelconque des revendications précédentes, dans laquelle la dispersion aqueuse comprend un plastifiant pour ajuster la dureté d'un film formé à partir de la résine utilisée comme liant ou comme agent d'encollage.

6. Feuille pour enregistrement à jet d'encre selon l'une quelconque des revendications précédentes, dans laquelle la dispersion aqueuse comprend 0,1 à 10% en poids d'un antioxydant, d'un absorbant UV ou d'un composé capable de réagir avec un colorant.

7. Feuille pour enregistrement à jet d'encre selon la revendication 6, dans laquelle l'antioxydant, l'absorbant UV ou le composé capable de réagir avec un colorant est contenu au moins dans une couche superficielle de la feuille pour enregistrement.

8. Feuille pour enregistrement à jet d'encre selon la revendication 6, dans laquelle l'antioxydant, l'absorbant UV ou le composé capable de réagir avec un colorant est contenu dans la feuille pour enregistrement.

9. Feuille pour enregistrement à jet d'encre selon la revendication 6, 7 ou 8, dans laquelle le composé capable de réagir avec un colorant est un acide phosphotungstique, un acide phosphomolybdique ou un acide phosphotungstomolybdique.

10. Feuille pour enregistrement à jet d'encre selon l'une quelconque des revendications précédentes, dans laquelle le rapport pondéral de la dite charge au dit agent liant est de 1:1 à 2:1.
